

June 7, 1960

C. MCKINLEY

2,939,778

LIQUID EXPLOSIVE

Filed June 21, 1956

5 Sheets-Sheet 1



INVENTOR  
CLYDE MCKINLEY

BY *James J. Flanery*  
ATTORNEY

June 7, 1960

C. MCKINLEY

2,939,778

LIQUID EXPLOSIVE

Filed June 21, 1956

5 Sheets-Sheet 2

SOLID-LIQUID EQUILIBRIA  
ETHANE - OXYGEN



MOLE. PERCENT OXYGEN  
IN ETHANE - OXYGEN

FIG. 5

SOLID-LIQUID EQUILIBRIA  
METHANE - OXYGEN



MOLE. PERCENT OXYGEN  
IN METHANE - OXYGEN

FIG. 4

INVENTOR

GLYDE MCKINLEY

BY

*Glyde McKinley*

ATTORNEY

June 7, 1960

C. MCKINLEY

2,939,778

LIQUID EXPLOSIVE

Filed June 21, 1956

5 Sheets-Sheet 3



FIG. 6

INVENTOR  
CLYDE MCKINLEY  
BY *James J. Sharley*  
ATTORNEY

June 7, 1960

C. MCKINLEY

2,939,778

LIQUID EXPLOSIVE

Filed June 21, 1956

5 Sheets-Sheet 4

OXYGEN-METHANE SYSTEM



FIG. 7

INVENTOR

CLYDE MCKINLEY

BY

*Jerry J. Shandley*

ATTORNEY

June 7, 1960

C. MCKINLEY

2,939,778

LIQUID EXPLOSIVE

Filed June 21, 1956

5 Sheets-Sheet 5

OXYGEN-ETHANE SYSTEM



FIG. 8

INVENTOR

CLYDE MCKINLEY

BY

*Clyde McKinley*

ATTORNEY

1

2,939,778

## LIQUID EXPLOSIVE

Clyde McKinley, Allentown, Pa., assignor to Air Products Incorporated, a corporation of Michigan

Filed June 21, 1956, Ser. No. 592,800

29 Claims. (Cl. 52--1)

This invention relates to explosives and more particularly to an explosive solution comprising fuel material dissolved in liquid oxygen. The invention further relates to the preparation, storage, and handling of such solutions, and to a method of producing an explosion.

Users of oxygen and others familiar with the art have long looked upon fuel-oxygen mixtures as being extremely hazardous and to be avoided wherever possible. This teaching of the art is understandable in view of numerous violent explosions experienced by those working in the art over the years, and to minimize the danger of explosion in instances where intimate contact between oxygen and a readily oxidizable fuel material is likely, elaborate safety precautions have been practiced. However, such safety precautions, generally speaking, have been limited to excluding oxygen from contact with a fuel material, or carefully controlling the oxygen concentration and the temperature of the fuel-oxygen mixture, or by limiting the quantity of fuel-oxygen mixture which is available at any given moment. For example, hydrocarbon lubricants are not employed as lubricants for compressors, valves, regulating devices, etc. handling oxygen gas, and thus, by excluding such fuel material from intimate contact with the oxygen, explosions may be prevented. In chemical processes wherein oxygen is an oxidant and the nature of the material to be oxidized is such that there is likelihood of an explosion, the concentration of oxygen and the temperature of the reaction mixture is carefully maintained within narrow limits in an effort to control the rate of reaction and thus prevent an explosion. Similarly, in certain other industrial applications, such as oxy-acetylene welding, the oxygen and acetylene are stored in separate cylinders and each gas is fed from its storage cylinder through a separate line to the welding torch where the two gases are mixed at the time of burning.

The foregoing is illustrative of teachings presently available in the art. It is apparent it has always been assumed that the hazards involved when oxygen is brought into intimate contact with a fuel material are prohibitive, and no teaching has been available heretofore as to how such hazards could be overcome, especially with large quantities of fuel-oxygen mixture and where the concentration of readily oxidizable fuel material in oxygen is relatively high. In fact, the art has never regarded the physical state of the fuel-oxygen mixture as important in reducing the hazard involved, or that fuel-oxygen mixtures could be prepared, stored and used in comparative safety.

The present invention resides in the discovery that solutions of fuel in liquid oxygen constitute a new and improved form of explosive which can be prepared, stored and used in relative safety under certain controlled conditions. More specifically, the present invention resides in the discovery that solutions of methane (or methane with small proportions of heavier normally gaseous hydrocarbons) in liquid oxygen constitute a new and improved form of explosive which can be prepared,

2

stored and used in relative safety under certain controlled conditions.

It is a principal object of the present invention to provide a novel explosive comprising a solution of fuel material dissolved in liquid oxygen.

It is a further object of the present invention to provide a novel method for the preparation, handling and storage of solutions containing a fuel material dissolved in liquid oxygen.

10 It is still a further object of the present invention to provide an improved package containing a solution of fuel material dissolved in liquid oxygen.

It is still a further object of the present invention to provide a novel method of producing an explosion 15 wherein an explosive charge comprising a solution of fuel material dissolved in liquid oxygen is exploded.

Still other objects of the present invention and the advantages thereof will become apparent to those skilled in the art by reference to the following detailed description 20 and the drawings, in which:

Fig. 1 is a diagrammatic sectional view taken through a package containing fuel material dissolved in liquid oxygen with means for refrigerating the solution;

Fig. 2 is a diagrammatic sectional view taken through 25 a package comprising a receptacle provided with two compartments, wherein one compartment contains liquid oxygen and the other compartment contains fuel material;

Fig. 3 diagrammatically illustrates one method of preparing, handling and storing a solution containing fuel 30 material dissolved in liquid oxygen;

Figs. 4, 5 and 6 are graphs illustrating solid-liquid equilibria for methane-oxygen, ethane-oxygen, and propane-oxygen systems, respectively;

Fig. 7 is a graph illustrating bubble point curves at 35 14.7, 50, 100 and 200 p.s.i.a. pressures for the oxygen-methane system plotted against temperature, together with partial pressure curves at 0.79, 2.7, 5.4 and 10.8 p.s.i. pressures for methane; and

Fig. 8 is a graph illustrating bubble point curves at 40 14.7, 50, 100 and 200 p.s.i.a. pressures for the oxygen-ethane system plotted against temperature, together with partial pressure curves at 0.60 and 2.05 p.s.i. pressures for ethane.

In accordance with one feature of the present invention, 45 a new and improved explosive is provided by dissolving a suitable fuel material in liquid oxygen in quantities sufficient to provide a solution which is explosive but not in quantities sufficient to precipitate from the resultant solution a solid phase or second immiscible liquid phase comprising fuel material.

The term "explosive" is used herein in the generic 50 sense, and is intended to include propellants and disruptives. Explosives of the invention characterized by a higher and more violent release of energy may be obtained by exploding a body of the solution after adjusting the fuel content of the solution to about stoichiometric proportions, while explosives characterized by a lower and less violent release of energy may be obtained by exploding a body of the solution after adjusting either the fuel or oxygen to a proportion lower than that required

55 for a stoichiometric solution. The release of energy in the use of the explosive of the present invention can be controlled by a different method, covered by copending application Serial No. 592,748, having the same filing date as the present application. Thus, the solutions described herein are explosives which may have characteristics varying over a wide range depending upon the concentration of fuel in the solution and the method of use.

60 The chemical nature of suitable fuel materials useful for the purpose of the present invention may vary widely provided the particular fuel material selected is suf-  
65

70 The chemical nature of suitable fuel materials useful for the purpose of the present invention may vary widely provided the particular fuel material selected is suf-

ficiently soluble in liquid oxygen under the controlled conditions to produce an explosive solution, and otherwise capable of being dissolved in liquid oxygen without appreciable hazard under the conditions taught herein. However, in accordance with the present invention, methane is the preferred fuel material and as such stands in a class by itself because of a combination of factors: notably, its high energy content coupled with its high solubility in liquid oxygen at atmospheric pressure and temperatures between the boiling and freezing points of liquid oxygen. With reference to Figs. 4 and 5 of the drawing, it may be noted that the solubility of saturated open chain hydrocarbons in liquid oxygen decreases rapidly with increasing molecular weight. For example, at  $-320^{\circ}$  F. the solubility of methane in liquid oxygen is about 75 mol percent, the solubility of ethane in liquid oxygen is about 10 mol percent and the solubility of propane in liquid oxygen (not shown) is about 5 mol percent. Thus while methane is the preferred fuel material, it is apparent that a mixture of methane, ethane and propane may be used. Natural gas, which is made up largely of methane together with small percentages of ethane and inconsequential amounts of higher saturated open chain hydrocarbons is an excellent fuel material for purposes of this invention.

Essentially pure liquid oxygen may be advantageous in some applications where a solution providing a maximum amount of available power per unit weight is desired. However, small amounts of nitrogen and inert gases which may be present in commercial liquid oxygen are not detrimental for the purposes of the present invention other than in possibly lowering the reaction rate slightly, or in necessarily requiring a greater weight of the impure liquid oxygen, and thus the resultant solution, to provide an equal amount of explosive energy.

The present invention will be described hereinafter with particular reference to methane as the fuel material, it being understood, as mentioned above, that other suitable fuels or mixtures of other suitable fuels with methane may be used.

It is generally desirable from the standpoint of safety to prepare solutions of methane in liquid oxygen in such a manner that a solid phase or "methane ice" is not precipitated. Thus in preparing the solutions of the invention, the liquid oxygen and the methane preferably should be brought together in such proportions that a homogeneous liquid mixture or solution consisting of a single liquid phase is maintained at all times and without a solid precipitate and/or a second immiscible liquid phase comprising methane being present therein. Otherwise, the hazard involved in preparing the solutions of the invention may be increased appreciably. However, it may be stated that this is not always essential and in some instances the solution may temporarily contain a precipitate and/or a second immiscible liquid phase during preparation which is later dissolved.

When the solution is held at a temperature below its boiling point, the vapor pressure of the solution will be less than atmospheric pressure and for this reason it may be desirable to supply an inert gas to the vapor phase above the solution in such quantities as to provide a pressure on the solution which is no less than atmospheric pressure. Suitable gases for this purpose include nitrogen and helium, with helium being preferred in instances where it is desired that the inert gas be substantially insoluble in the solution. The inert gas may be supplied at a pressure substantially greater than atmospheric and thus provide a means for forcing the solution from a container, as well as maintaining the vapor phase above the solution noninflammable.

It is part of the present invention, from the standpoint of reducing the hazard involved in preparing, handling and storing the solutions described herein, to maintain the composition of the vapor phase above the solution noninflammable. Mixtures of methane and oxygen in the vapor phase and at atmospheric pressure are inflamm-

mable when methane is present in concentrations varying between 5.4 mol percent and 59.2 mol percent; while mixtures of methane and air under the same conditions are inflammable if methane is present in concentrations between about 5 mol percent and 15 mol percent. The lower inflammability limit for mixtures of ethane and oxygen in the vapor phase and at atmospheric pressure is 4.1 mol percent, while the upper limit is 50.5 mol percent. With an increase in pressure, the lower inflammability limit in each instance is lowered only slightly, while the upper limit in each instance is raised somewhat. By maintaining the composition of the methane-oxygen vapor phase above the solution at a concentration of methane which is noninflammable, the likelihood of explosion in the highly sensitive vapor phase will be greatly reduced or may even be eliminated. As pointed out above, an unobvious feature of the present invention is the lack of sensitivity of the solution of methane in liquid oxygen. Thus under proper vapor phase conditions, or no vapor phase, the solution may be rendered safe.

In accordance with the present invention, the concentration of methane in the vapor phase may be controlled by a number of methods. One such method comprises maintaining the concentration of methane in liquid oxygen at such a level and the temperature of the resultant solution low enough so as to provide a noninflammable mixture of vapor in equilibrium with the solution. For example, applicant has found that a solution containing stoichiometric quantities of methane, i.e., about 33 mol percent methane, has noninflammable vapor in equilibrium with the solution at temperatures up to about  $-291.5^{\circ}$  F., and by refrigerating the solution so as to maintain it below this temperature the vapor phase may be rendered safe. However, referring to Fig. 4 of the drawings, it may be seen that solid methane will begin to precipitate from a solution containing 33 mol percent methane at about  $-348^{\circ}$  F., and it follows that the temperature of this solution should preferably be maintained in a range above about  $-348^{\circ}$  F. and below about  $-291.5^{\circ}$  F. so as to provide a solution free of precipitated methane ice and with a noninflammable vapor phase. Inasmuch as the vapor pressures of both oxygen and methane are well known at varying temperatures, as well as the manner of calculating the mol percent composition of a vapor phase in equilibrium with a solution of known mol percent composition, it follows that one skilled in the art may readily determine the upper temperature limit which any given solution of known composition may not exceed in order to provide a noninflammable vapor phase in equilibrium with the solution. Likewise, one skilled in the art, by reference to Fig. 4, may readily determine the lower temperature limit, i.e., the lowest temperature at which any given solution is free of precipitated methane ice. The temperature of solutions in accordance with the present invention are preferably maintained between the foregoing upper and lower temperature limits. Even better results from the standpoint of safety are possible by maintaining the solutions at a temperature about half way between the above mentioned upper and lower temperature limits. Usually the most practical refrigerant for this purpose, provided the solution contains no more than about 70 mol percent methane, is liquid nitrogen under atmospheric pressure.

Another method of rendering the vapor phase noninflammable, even though the concentration of methane and the temperature of the solution is such that normally the vapor phase in equilibrium with the solution would be inflammable, is by supplying a gaseous diluent to the normally inflammable vapor phase. The gaseous diluent is supplied to the vapor phase in quantities sufficient to provide a noninflammable vapor phase, and preferably in such a manner as to flow at least a portion of the diluent along the surface of the solution for the purpose of preventing the temporary formation of a

localized inflammable mixture of vapors near the surface of the solution. The term "gaseous diluent" as used in the specification and claims is intended to include gaseous materials or mixtures, including oxygen, which are at least no more reactive with methane under the conditions employed herein than is oxygen. The particular gaseous diluent employed may be any suitable gaseous substance which will render the vapor mixture noninflammable by reason of its inert properties under the conditions employed, such as nitrogen, or it may be a gas which simply dilutes the vapor mixture to such a level as to give a noninflammable mixture, such as where sufficient air or oxygen is supplied to yield a noninflammable mixture. The source of gaseous diluent may be auxiliary in nature, that is supplied from a source outside the solution, or it may be supplied from the solution itself, as in instances where a relatively small mol fraction of methane is dissolved in a relatively large mol fraction of liquid oxygen with the resultant vapor composition being sufficiently high in oxygen and low in methane as to be rendered noninflammable. A third material such as nitrogen may be present in the solution for this purpose, as well as for the purpose of rendering the solution less sensitive.

Still another method of rendering the vapor phase noninflammable is by providing a floating film or follower for the surface of the solution, thereby preventing or at least greatly reducing vaporization. This may be accomplished by a number of methods, such as by providing a thin plastic sheet in contact with the entire surface of the solution, or by covering the surface of the solution with a layer of minute plastic bubbles of a type commercially available for such purpose. Of course a rigid impervious structure, where practical will accomplish the desired result. The terms "follower" and "floating follower" where they appear in this specification and claims are intended to mean a thin plastic sheet, or a coating of minute plastic bubbles, rigid structure, or equivalent, as above described. The vapor pressure apparently exhibited by the solution may be "lowered" by the foregoing procedure and the term "effective vapor pressure of the solution" where it appears in this specification and claims is intended to mean the vapor pressure of a solution after being "lowered" in this or similar manner, or the normal vapor pressure of a solution not provided with a follower or floating follower.

It is obvious that a combination of two or more of the above described methods for rendering the vapor phase of the solution noninflammable may be of advantage in many instances. Likewise, equivalents may be substituted along the lines of other well known methods.

The concentration of methane in liquid oxygen may vary over wide ranges. For example, the lower limit may be generally stated as that concentration of methane in liquid oxygen yielding a resultant solution which is explosive, while the upper limit is somewhat dependent upon the temperature of the solution and may be determined by reference to Fig. 4, but in any event the concentration is not sufficiently high as to cause a solid precipitate comprising methane to be formed therein. For example, at -320° F., the composition of the resultant solution may vary between about 5 mol percent methane and about 75 percent methane. A solution containing about stoichiometric quantities of methane will provide an explosive having a maximum amount of energy available per unit weight of solution. Solutions containing a concentration of either oxygen or methane in excess of stoichiometric proportions will provide a solution having less energy available per unit weight of solution. Thus the properties of the explosive may be varied somewhat by varying the concentration of methane, with the explosive being most violent at about stoichiometric proportions and decreasing in violence when either the methane or oxygen is present in excess of stoichiometric proportions. Generally, solutions con-

taining between 5 mol percent methane and 50 mol percent methane are desirable explosives. Solutions containing less than 5 mol percent methane do not usually have sufficient power, while there appears to be no economic advantage as an explosive in going above 50 mol percent. For most applications, such as in mining operations, solutions containing between 25 and 50 mol percent methane give best results. In instances where a maximum amount of power per unit weight of solution is desired, a solution containing about stoichiometric quantities of methane, i.e., about 33 mol percent, is preferred.

Fig. 1 diagrammatically illustrates one suitable arrangement for storing or packaging the solutions of the present invention. The receptacle 1 is provided with an inlet 4 covered by a loosely fitting cap 3 and contains a solution 2 of methane in liquid oxygen. The receptacle 1 is immersed in liquid nitrogen refrigerant 5, which fills insulated container 6 to a desired level. While the refrigerant is specifically shown as liquid nitrogen under atmospheric pressure, the liquid nitrogen may be evaporated under vacuum if additional cold is desired, or other suitable liquefied gas refrigerants may be used. Means for controlling the composition of the vapor phase above solution 2, such as the various means previously discussed herein or as diagrammatically illustrated in Fig. 3, may be included if desired.

Fig. 2 diagrammatically illustrates one suitable arrangement for packaging fuel and liquid oxygen where by the solutions described herein may be prepared, stored, and used in safety. The insulated receptacle 7 is provided with a frangible partition 8 dividing receptacle 7 into an upper compartment 9 and a lower compartment 10. Upper compartment 9 is provided with an inlet 11 for filling compartment 9 with the liquid oxygen 12. A rigid tube 14 extends into compartment 9 of receptacle 7 through a flanged opening 15 which receives tube 14 in relatively movable relation. Tube 14 extends downwardly into compartment 10 through opening 16 in partition 8 thereby allowing compartment 10 to be filled with the liquid methane 17. Loosely fitting caps 18 and 19 cover inlet 11 and the outer end of tube 14, respectively. The frangible partition 8 is rigidly attached to tube 14. Tube 14 also extends upwardly and above inlet 11 a considerable distance so as to allow a falling weight or other force to drive tube 14 downwardly a sufficient distance to break frangible partition 8 without crushing receptacle 7.

When using receptacle 7, the lower compartment 10 is filled with the desired quantity of liquid methane 17 through tube 14 and cap 19 is snapped into place. Then compartment 9 is filled through inlet 11 with the desired quantity of liquid oxygen 12 and cap 18 snapped into place. The solution of methane in liquid oxygen may now be prepared safely by merely dropping a weight onto the upper end of tube 14, or otherwise applying sufficient force thereto, to drive tube 14 downwardly a distance sufficient to break frangible partition 8 without damaging receptacle 7. Compartment 9 is now in communication with compartment 10 and the liquid oxygen 12, being of a much higher specific gravity than methane, is free to flow downwardly mixing with the liquid methane 17 and thereby forming a solution of methane in liquid oxygen.

Fig. 3 diagrammatically illustrates one very satisfactory arrangement for and method of preparing relatively large quantities of a solution containing methane dissolved in liquid oxygen. A first receptacle 20 containing liquid methane 21 is provided with an inlet 22 covered by a loosely fitting cap 23 and an outlet 24 leading into storage tank 25. A second receptacle 26 containing liquid oxygen 27 is provided with an inlet 28 covered by a loosely fitting cap 29 and an outlet 30 leading to storage tank 25. The receptacles 20 and 26 and storage tank 25 are preferably provided with a source of refriger-

ation (not shown) which may be arranged in the manner shown in Fig. 1. The storage tank 25 is also provided with an inlet 33 and outlet 34 for supplying gaseous diluent to the vapor phase 31 above solution 32.

As mentioned above, it is generally desirable to provide refrigeration for receptacles 20 and 26 and storage tank 25. Preferably, liquid methane 21 should be cooled to a temperature only slightly above its freezing point and liquid oxygen 27 to a temperature of about  $-320^{\circ}$  F., or to a somewhat lower temperature if it is desired to produce solution 32 at a temperature of  $-320^{\circ}$  F. Liquid oxygen is a satisfactory refrigerant for liquid methane 21, while liquid nitrogen is the preferred refrigerant for both liquid oxygen 27 and solution 32. The solution 32 is preferably prepared by adding desired quantities of subcooled liquid methane 21 and liquid oxygen 27 to storage tank 25 via outlets 24 and 30 while supplying a gaseous diluent, such as nitrogen, to the vapor phase 31 via inlet 33 and outlet 34 and in quantities sufficient to provide a noninflammable vapor phase.

The solutions described herein provide an improved method of producing an explosion. A number of different variations are possible in the foregoing method as specifically applied to mining operations. For example, referring to Fig. 1, a blasting cap or the like may be attached to receptacle 1 containing solution 2 and then receptacle 1 is lowered into a hole previously drilled for this purpose. A suitable packing may then be applied above receptacle 1 and the blasting cap is detonated, thereby exploding solution 2. Alternatively, referring now to Fig. 2, a blasting cap or the like may be attached to insulated receptacle 7 containing liquid oxygen 12 and liquid methane 17, and the package lowered into a hole previously drilled. A weight can be dropped onto tube 14 to break partition 8 thus allowing the contents to mix and form a solution. The package is then ready to explode by means of the blasting cap. It is also possible to vary the above by filling an insulated receptacle by means of a hose or the like with either liquid oxygen or liquid methane, or both, after lowering the receptacle provided with an attached blasting cap into the hole. A receptacle for the solution may not always be necessary. For example, in some instances where a dry hole or a dry natural crevice is available, a blasting cap may be lowered to the bottom of the hole or crevice and the solution then added and exploded shortly thereafter. In instances where it is desired to prepare a number of the above described explosive charges and over a relatively long period of time, or under conditions where other refrigerant is not practical or available, it may be desirable to use solutions containing as little as about 5 mol percent methane. Such solutions may be allowed to "age" for three hours or more during which time the more volatile evaporating oxygen provides refrigeration and the methane content gradually increases to about 18 mol percent or higher. After a desired period of time, the remaining solution is exploded in the usual manner.

Referring now to Fig. 4 of the drawings which illustrates solid-liquid equilibria for methane and oxygen mixtures, it may be seen that a methane-oxygen mixture containing 40 mol percent methane and maintained at a temperature below about  $-363^{\circ}$  F. will consist of solid methane and solid oxygen. Upon warming to a temperature between about  $-363^{\circ}$  F. and  $-344^{\circ}$  F., this mixture will comprise solid methane in equilibrium with liquid methane-oxygen solution, and at temperatures above about  $-344^{\circ}$  F. and below its boiling point, the mixture consists of a homogeneous liquid mixture or solution of methane in oxygen which is free of a second liquid phase or solid precipitate comprising methane. Thus, it is apparent that the minimum temperature at which a methane-oxygen solution of the invention having a desired methane content can be maintained will be in the area above line 4A of the graph of Fig. 4. The max-

imum temperature is preferably a temperature below the boiling point of the solution at the pressure present and may be determined by reference to Fig. 7.

Referring now to Fig. 7 of the drawings, the bubble point curves 7A, 7B, 7C and 7D at 14.7, 50, 100 and 200 p.s.i.a. pressures, respectively, for the oxygen-methane system are plotted against temperature in the graph. The bubble point curves represent the isobaric equilibrium composition of the liquid mixture and were obtained by considering the oxygen-methane system an ideal solution. Thus, the bubble point curves represent the temperature and pressure at which the first bubble would form in a liquid mixture of a particular indicated composition as that mixture is gradually heated to a higher temperature. For example, a methane-oxygen liquid mixture containing 0.40 mol fraction or 40 mol percent of methane and held at a total pressure of 14.7 p.s.i.a. would be entirely liquid at temperatures within the range appearing on the graph below about  $-290^{\circ}$  F. and would have the first trace or bubble of vapor form at that temperature. It will be apparent that if this particular system is held at 14.7 p.s.i.a. and warmed to its boiling point, further evaporation takes place in such a way that the composition of the system moves along the bubble point curve 7A to higher temperatures and to higher compositions of methane. Since the lower limit of inflammability for methane-oxygen gaseous mixtures is 5.4 mol percent methane, the maximum allowable partial pressure of methane for a noninflammable mixture is less than 0.79, 2.7, 5.4 and 10.8 p.s.i. for gaseous oxygen-methane mixtures maintained under pressures of 14.7, 50, 100 and 200 p.s.i.a., respectively. Thus, the partial pressure curves 7(a), 7(b), 7(c) and 7(d) for methane represent the lower limit of inflammability for the methane-oxygen system when maintained under pressures of 14.7, 50, 100 and 200 p.s.i.a., respectively. For example, whenever the methane partial pressure in the vapor phase is under 0.79 p.s.i. with a total pressure of 14.7 or above on the system, the vapor phase mixture is below the lower inflammability limit. Similarly, any points under methane partial pressures of 2.7, 5.4 and 10.8 p.s.i. and at or above total pressures of 50, 100 and 200 p.s.i.a., respectively, are below the lower inflammability limits. Thus, the conditions required for a noninflammable vapor in equilibrium with the liquid methane-oxygen solution of desired composition may be readily determined from the foregoing.

Referring now to Fig. 5 of the drawings, which illustrates solid-liquid equilibria for ethane and oxygen mixtures, it may be seen that an ethane-oxygen mixture containing 40 mol percent ethane and maintained at a temperature below about  $-363^{\circ}$  F. will consist of solid ethane and solid oxygen. Upon warming, this mixture will comprise solid ethane in equilibrium with liquid ethane-oxygen solution at temperatures between about  $-363^{\circ}$  F. and  $-308^{\circ}$  F.; liquid ethane rich ethane-oxygen solution in equilibrium with oxygen rich liquid ethane-oxygen solution at temperatures between about  $-308^{\circ}$  F. and  $-298^{\circ}$  F.; and a homogeneous liquid mixture or solution of ethane in oxygen which is free of a second liquid phase or solid precipitate comprising ethane at temperatures above about  $-298^{\circ}$  F. and below the boiling point of the solution. Thus, it is apparent that the minimum temperature at which an ethane-oxygen solution of the invention having a desired ethane content is maintained will be in the area above line 5A of the graph of Fig. 5. The maximum temperature is preferably a temperature below the boiling point of the solution at the pressure employed and may be determined by reference to Fig. 8.

Referring now to Fig. 8 of the drawings, the bubble point curves 8A, 8B, 8C and 8D at 14.7, 50, 100 and 200 p.s.i.a. pressures, respectively, for the oxygen-ethane system are plotted against temperature in the graph. The bubble point curves represent the isobaric equilibri-

um composition of the liquid mixture and were obtained by considering the oxygen-ethane system an ideal solution. The bubble point curves thus represent the temperature and pressure at which the first bubble would form in a liquid mixture of a particular indicated composition as that mixture is gradually heated to a higher temperature. For example, an ethane-oxygen liquid mixture containing 0.40 mol fraction or 40 mol percent of ethane and held at a total pressure of 50 p.s.i.a would be entirely liquid at temperatures below about  $-260^{\circ}$  F. and would have the first trace or bubble of vapor form at that temperature. It will be apparent that if this particular system is held at 50 p.s.i.a. and warmed to its boiling point, further evaporation takes place in such a way that the composition of the system moves along the bubble point curve 8A to higher temperatures and to higher compositions of ethane. Since the lower limit of inflammability for ethane-oxygen gaseous mixtures is 4.1 mol percent ethane, the maximum allowable partial pressure of ethane for a noninflammable mixture is less than 0.60 and 2.05 p.s.i. for gaseous ethane-oxygen mixtures maintained under pressures of 14.7 and 50 p.s.i.a, respectively. Thus the partial pressure curves 8(a) and 8(b) for ethane represent the lower limit of inflammability for a gaseous oxygen-ethane system when maintained at pressures of 14.7 and 50 p.s.i.a., respectively. It will be apparent that any point under an ethane partial pressure of 0.60 p.s.i. and at or above 14.7 p.s.i.a. total pressure on the system is below the lower inflammability limit. Similarly, any point under an ethane partial pressure of 2.05 and at or above a total pressure of 50 p.s.i.a. is below the lower inflammability limit. It follows that the conditions required for a noninflammable vapor above the liquid ethane-oxygen may be readily determined from the foregoing.

Fig. 6 illustrates solid-liquid equilibria for propane and oxygen mixtures. Applicant lacks data above  $-290^{\circ}$  F. and the portions of curve 6A between  $-290^{\circ}$  F. and  $-270^{\circ}$  F. indicate reasonable extrapolation. The remainder of the loop of curve 6A above  $-270^{\circ}$  F., constitutes a mere guess at the nature of this portion of the curve as it is based on the slopes of the portions below  $-270^{\circ}$  F. Actually, it may not be possible to raise the temperature of the propane-oxygen system high enough to obtain a single liquid phase in the region of the curve 6A above  $-270^{\circ}$  F. It may be that the two phases will persist up to the critical temperature of the mixture, under which conditions a gaseous phase must necessarily exist. It may be seen from Fig. 6 that a propane-oxygen mixture containing 40 mol percent propane and maintained at a temperature below about  $-363^{\circ}$  F. will consist of solid propane and solid oxygen. Upon warming to temperatures between about  $-363^{\circ}$  F. and about  $-270^{\circ}$  F., this mixture will comprise solid propane in equilibrium with liquid propane-oxygen solution. At higher temperatures, phase conditions are unknown but it seems reasonable to assume that a single phase solution cannot exist except at relatively high temperatures. On the other hand, a propane-oxygen mixture containing 5 mol percent propane can be a single phase liquid solution at  $-300^{\circ}$  F.

Proper interpretation of Figs. 4 through 8 of the drawings will readily provide conditions necessary for the preparation, storage and use of preferred explosives of the nature described herein. For example, should it be desirable to prepare a methane-oxygen solution containing 40 mol percent methane, the minimum temperature at which such a solution exists free of a precipitate comprising methane may be determined from the graph of Fig. 4 to be about  $-344^{\circ}$  F. Then by referring to curve 7A of Fig. 7, the boiling point of a methane-oxygen solution containing 0.40 mol fraction or 40 mol percent of methane will be found to be about  $-290^{\circ}$  F. at a pressure of 14.7 p.s.i.a. Thus the solution may be held at a temperature above  $-344^{\circ}$  F. but below  $-290^{\circ}$  F.

and at a pressure of at least one atmosphere. However, since a noninflammable vapor in equilibrium with the solution is desirable, it may be seen from the partial pressure curve for methane 7(a) that the temperature of the solution should be below about  $-294^{\circ}$  F. in order to not exceed the lower inflammability limit and maintain a noninflammable vapor phase. In actual practice, a temperature about halfway between the minimum temperature and the temperature at which the lower inflammability limit is exceeded for the particular composition is preferred. When the solution is held at a temperature sufficiently high to cause the lower inflammability limit to be exceeded, it is necessary to resort to a gaseous diluent or other means described herein to maintain the vapor phase noninflammable.

Similarly, if an ethane-oxygen solution containing 40 mol percent ethane is desired, the minimum temperature at which such a liquid solution exists free of a second liquid phase or precipitate comprising ethane may be determined to be about  $-298^{\circ}$  F. from the graph of Fig. 5. Then by referring to curves 8A and 8B of Fig. 8, the boiling point of an ethane-oxygen solution containing 0.40 mol fraction or 40 mol percent of ethane will be found to be about  $-288^{\circ}$  F. and  $-260^{\circ}$  F. at pressures of 14.7 and 50 p.s.i.a., respectively. Since the minimum temperature is  $-298^{\circ}$  F. and the boiling point of the solution at atmospheric pressure is  $-288^{\circ}$  F., a pressure in excess of atmospheric must be resorted to in order to have a boiling point sufficiently higher than the minimum temperature of  $-298^{\circ}$  F. to permit practical operation. Assuming the selection of a pressure of 50 p.s.i.a., the solution may be held at a temperature above the minimum temperature of  $-298^{\circ}$  F. and below its boiling point of  $-260^{\circ}$  F. It may be seen from the partial pressure curve for ethane 8(b) that this temperature range is sufficiently low so as not to exceed the lower inflammability limit and to maintain the vapor phase in equilibrium with the solution noninflammable, even at its boiling point.

Inspection of Fig. 6 shows that propane as the sole fuel, i.e., in substantial proportions, can be maintained in single phase solution in oxygen, if at all, only at high temperatures and therefore high pressures. In small proportions, as in mixtures with methane and ethane, propane can be used at lower temperatures and pressures and in such case the inflammability of the vapor phase is not critically affected by the propane.

A solution containing stoichiometric or higher proportions of a fuel material dissolved in liquid oxygen and which is free of a second liquid phase or precipitate comprising fuel material may be prepared in many instances using fuels such as ethane or propane which are not normally soluble in oxygen to the desired extent at the low temperatures necessary for handling the solution at atmospheric pressure. It is possible to provide a mixture including ethane, propane, or other suitable fuel and liquid oxygen which normally exhibits at or near atmospheric pressure a second liquid phase or precipitate comprising fuel material and by increasing the temperature of the mixture while simultaneously increasing the pressure to at least the vapor pressure of the mixture at its particular temperature, it is possible to maintain the mixture as a solution free of a second liquid phase or precipitate comprising fuel material. This is of importance in applications where it is not necessary to control the temperature of the mixture in order to control the hazard involved. In such instances, it may be possible to place the mixture in a closed vessel and allow the temperature to rise to a temperature under the critical temperature for the mixture, and thereby produce a solution suitable for the purposes of the invention. Where closed pressure vessels are desirable, the fuel material will be a compound or mixture of compounds which will dissolve in the desired proportions in the liquefied oxygen at the pressure and temperature employed.

A solution of fuel in liquid oxygen has been found to

be a much more efficient explosive than two phase liquid mixtures of oxygen and fuel, or suspensions of fuel in liquid oxygen. The increase in efficiency is thought to be due to the intimate molecular relationship of fuel and oxygen which exists in such solutions. Thus upon explosion of the solution, all available energy may be fully released and in a minimum period of time.

The following examples further illustrate certain features of the present invention.

*Example I*

A standard blasting cap was fastened to the outer surface of a short section of bright copper tubing and the copper tubing together with the blasting cap immersed in liquid nitrogen. The blasting cap was then detonated and the copper tubing recovered for purposes of examination.

Upon examination of the copper tubing, only a very minor surface area was found to be damaged or discolored.

*Example II*

A solution containing 33 mol percent methane in liquid oxygen was prepared by liquefying a mixture of gaseous methane and oxygen.

15 cc. of the above solution was placed in a short section of bright copper tubing which was closed off at one end and provided with a standard commercial blasting cap fastened to the outer surface of the tube. The copper tubing containing the solution together with the blasting cap was immersed in liquid nitrogen. The tubing, blasting cap, manner of fastening the blasting cap and immersion in liquid nitrogen was identical with that of Example I.

Upon detonation of the blasting cap, the solution exploded violently causing considerable damage to the immediate surrounding area. Small portions of copper tube found in the debris were brittle and exhibited numerous fissures.

*Example III*

A "matchhead," which is a term commonly used for a commercially available device for initiating explosions and characterized by heat release only as compared with the heat and detonating effect of a standard blasting cap, was fastened to the outer surface of a section of bright copper tubing identical with that of Example II. Then 15 cc. of the solution described in Example II was placed in the copper tubing and the same immersed in liquid nitrogen as in the foregoing examples.

The matchhead was then fired, but the solution failed to explode. The above procedure was followed several times with identical results.

The above procedure was modified by fastening the matchhead inside the tubing and within the solution. The solution again failed to explode, although examination of the matchhead showed it had fired.

It is apparent from this experiment that a stoichiometric solution of methane in liquid oxygen is relatively safe provided the temperature of the solution is such as to provide a noninflammable vapor phase in equilibrium with the solution.

*Example IV*

A spark plug was arranged in a flask so as to be slightly above the surface of solution after addition of 15 cc. of solution. Then 15 cc. of the solution described in Example II was added to the flask, and the flask immersed in a small quantity of liquid nitrogen.

The spark plug was then "sparked" for about 5 minutes before an explosion occurred. At the time of explosion, the liquid nitrogen had boiled down and no longer covered the solution.

It is apparent from the foregoing the vapor phase in equilibrium with a stoichiometric solution of methane in liquid oxygen is noninflammable provided the tempera-

ture of the solution is maintained at or below the boiling point of liquid nitrogen, i.e., about -320° F.

In the instances where it may be desirable, the explosive of the present invention may contain effective quantities of an additive such as an inhibitor or promoter for the purpose of modifying the characteristics thereof and thereby provide an explosive even more effective in a specific application. Additionally nitrogen, liquid air, etc. added to the solution as described above not only controls the sensitivity of the vapor phase but is useful in controlling the sensitivity of the solution.

The foregoing detailed description and the specific examples are for the purpose of illustration only, and are not intended as limiting to the scope or spirit of the appended claims.

What is claimed is:

1. An explosive consisting essentially of at least one fuel material selected from the class consisting of methane, ethane and propane dissolved in liquid oxygen in an amount to produce an explosive and prevent the formation of a second nongaseous phase comprising fuel material and having a noninflammable vapor phase above the resulting solution, the solution of fuel material in liquid oxygen containing up to about 75 mol percent of methane, up to about 40 mol percent of ethane and up to about 7 mol percent of propane and having a temperature below the critical temperature of the resultant solution and above -363° F. and the noninflammable vapor phase above the solution containing less than 5.4 mol percent of fuel material.
2. An explosive consisting essentially of methane dissolved in liquid oxygen in an amount to produce an explosive and prevent the formation of a second nongaseous phase comprising methane and having a noninflammable vapor phase above the resulting solution, the solution of methane dissolved in liquid oxygen containing 5-75 mol percent of methane and having a temperature below its critical temperature and above -363° F. and the noninflammable vapor phase above the solution containing less than 5.4 mol percent of methane.
3. An explosive in accordance with claim 2 wherein the concentration of methane is about 33 mol percent.
4. A package comprising a contained body consisting essentially of liquid oxygen having dissolved therein a fuel material selected from the class consisting of methane, ethane and propane in an amount to produce an explosive and prevent the formation of a second non-gaseous phase comprising fuel material, the body of fuel material and liquid oxygen containing up to about 75 mol percent methane, up to about 40 mol percent ethane and up to about 7 mol percent propane, a contained body of liquefied gas refrigerant surrounding the first claimed body, the refrigerant having a boiling point under the existing pressure not greater than the boiling point of the first claimed body, the pressure on the surface of the body of oxygen and fuel material and the pressure on the surface of the body of refrigerant being such that the body of refrigerant has a temperature lower than the boiling point of the body of oxygen and fuel and such as to maintain the composition of the vapor above the surface of the body of oxygen and fuel noninflammable, the temperature of the body being maintained below its critical temperature and above -363° F. and the vapor containing less than 5.4 mol percent of fuel material.

5. A package comprising a contained body consisting essentially of liquid oxygen having methane dissolved therein in effective amount to form an explosive but not in a concentration sufficiently high to precipitate a solid phase comprising methane, the body of methane and liquid oxygen containing 5-75 mol percent methane a contained body of liquefied gas refrigerant surrounding the first claimed body, the refrigerant having a boiling point under the existing pressure not greater than the boiling point of oxygen, the pressure on the surface of the body of oxygen and methane and the pressure on the

surface of the body of refrigerant being such that the body of refrigerant has a temperature lower than the boiling point of the body of oxygen and methane and such as to maintain the composition of the vapor phase above the surface of the body of oxygen and methane noninflammable, the temperature of the body of liquid oxygen and methane being maintained below its critical temperature and above  $-363^{\circ}$  F. and the vapor phase containing less than 5.4 mol percent of methane.

6. The package of claim 5 wherein the refrigerant is nitrogen.

7. The package of claim 5 wherein the concentration of methane in liquid oxygen is about 33 mol percent.

8. A package comprising a contained body consisting essentially of liquid oxygen having dissolved therein at least one fuel material selected from the class consisting of methane, ethane and propane, the fuel material being present in the liquid oxygen in effective amount to form an explosive but not in a concentration sufficiently high to precipitate a second nongaseous phase comprising fuel material, the body of fuel material and liquid oxygen containing up to about 75 mol percent methane, up to about 40 mol percent ethane and up to about 7 mol percent propane, a contained body of liquefied gas refrigerant surrounding the first claimed body, the refrigerant having a boiling point under the existing pressure not greater than the boiling point of the first claimed body, the pressure on the surface of the body of oxygen and fuel and the pressure on the surface of the body of refrigerant being such that the body of refrigerant has a temperature lower than the boiling point of the body of oxygen and fuel, and means for supplying a gaseous diluent above the surface of the body of oxygen and fuel at a rate sufficient to maintain the composition of the vapor phase above the body of oxygen and fuel noninflammable, the temperature of the body of liquid oxygen and fuel material being maintained below its critical temperature and above  $-363^{\circ}$  F. and the concentration of the fuel in the vapor phase at less than 5.4 mol percent.

9. A package comprising a contained body consisting essentially of liquid oxygen having methane dissolved therein in effective amount to form an explosive but not in a concentration sufficiently high to precipitate a solid phase comprising methane, the body of methane and liquid oxygen containing 5-75 mol percent methane a contained body of liquefied gas refrigerant surrounding the first claimed body, the refrigerant having a boiling point under the existing pressure not greater than the boiling point of oxygen, the pressure on the surface of the body of oxygen and methane and the pressure on the surface of the body of refrigerant being such that the body of refrigerant has a temperature lower than the boiling point of the body of oxygen and methane, and means for supplying a gaseous diluent above the surface of the body of oxygen and methane at a rate sufficient to maintain the composition of the vapor phase above the body of oxygen and methane noninflammable, the temperature of the body of methane and liquid oxygen being maintained below its critical temperature and above  $-363^{\circ}$  F. and the concentration of methane in the vapor phase at less than 5.4 mol percent.

10. The package of claim 9 wherein the refrigerant and the gaseous diluent comprise nitrogen.

11. The package of claim 9 wherein the concentration of methane in the liquid oxygen is about 33 mol percent.

12. A package comprising a receptacle containing a body consisting essentially of liquid oxygen having at least one fuel material selected from the class consisting of methane, ethane and propane dissolved therein, the fuel material being present in the liquid oxygen in effective amount to form an explosive but not in a concentration sufficiently high to precipitate a second nongaseous phase comprising fuel material, the body of fuel material and liquid oxygen containing up to about 75 mol percent methane, up to about 40 mol percent ethane and up to

about 7 mol percent propane, and means for supplying a gaseous diluent above the surface of the body of liquid oxygen and fuel material at a rate sufficient to maintain the composition of the vapor phase above the body of liquid oxygen and fuel material noninflammable, the body of liquid oxygen and fuel material having a temperature below its critical temperature and above  $-363^{\circ}$  F. and the vapor phase containing less than 5.4 mol percent fuel material.

10. 13. The package of claim 12 wherein the gaseous diluent comprises nitrogen.

14. A package comprising a receptacle containing a body consisting essentially of liquid oxygen having methane dissolved therein in effective amount to form an explosive but not in a concentration sufficiently high to precipitate a solid phase comprising methane, the body of methane and oxygen containing 5-75 mol percent methane, and means for supplying a gaseous diluent above the body of liquid oxygen and methane at a rate sufficient to maintain the composition of the vapor phase above the body of liquid oxygen and methane noninflammable, the body of liquid oxygen and methane having a temperature below its critical temperature and above  $-363^{\circ}$  F. and the vapor phase containing less than 5.4 mol percent methane.

15. 15. The package of claim 14 wherein the gaseous diluent comprises nitrogen.

16. A package comprising a receptacle containing a body consisting essentially of liquid oxygen having at least one fuel material selected from the class consisting of methane, ethane and propane dissolved therein in effective amount to form an explosive but not in a concentration sufficiently high to precipitate a second nongaseous phase comprising fuel material, the body of fuel material and liquid oxygen containing up to about 75 mol percent methane, up to about 40 mol percent ethane and up to about 7 mol percent propane, and the surface of the body of liquid oxygen and fuel material having a follower thereon selected from the class consisting of minute plastic bubbles and thin plastic sheets to maintain the composition of the vapor phase above the body of liquid oxygen and fuel noninflammable, the temperature of the body of liquid oxygen and fuel material being below its critical temperature and above  $-363^{\circ}$  F. and the concentration of fuel material in the vapor phase being less than 5.4 mol percent.

17. A package comprising a receptacle containing a body consisting essentially of liquid oxygen having methane dissolved therein in effective amount to form an explosive but not in a concentration sufficiently high to precipitate a second nongaseous phase comprising methane, the body of liquid oxygen and methane containing 5-75 mol percent methane, and the surface of the body of liquid oxygen and methane having a follower thereon selected from the class consisting of minute plastic bubbles and thin plastic sheets to maintain the composition of the vapor phase above the body of liquid oxygen and methane noninflammable, the temperature of the body of liquid oxygen and methane being below its critical temperature and above  $-363^{\circ}$  F. and the concentration of methane in the vapor phase being less than 5.4 mol percent.

18. The method of preparing a solution consisting essentially of at least one fuel material selected from the class consisting of methane, ethane and propane dissolved in liquid oxygen which comprises dissolving the fuel material in the liquid oxygen in an amount effective to produce an explosive and prevent formation of a second nongaseous phase comprising fuel material while maintaining the composition of the vapor phase above the resultant solution noninflammable, the resultant solution containing up to 75 mol percent methane, up to 40 mol percent ethane and up to 7 mol percent propane and the concentration of fuel material in the vapor phase being less than 5.4 mol percent, the temperature of the

65 70 75

resultant solution being maintained below its critical temperature and above  $-363^{\circ}$  F. and the pressure being at least equal to the effective vapor pressure of the resultant solution at its temperature.

19. The method of preparing a solution consisting essentially of methane dissolved in liquid oxygen which comprises dissolving the methane in liquid oxygen in an amount effective to produce an explosive and prevent formation of a second nongaseous phase comprising fuel material while maintaining the composition of the vapor phase above the resultant solution of methane in liquid oxygen noninflammable, the resultant solution containing 5-75 mol percent methane and the concentration of methane in the vapor phase being less than 5.4 mol percent, the resultant solution being maintained below its critical temperature and above  $-363^{\circ}$  F. and the pressure being at least equal to the effective vapor pressure of the resultant solution at its temperature.

20. The method of claim 19 wherein the composition of the vapor above the resultant solution is maintained at a noninflammable composition by supplying a gaseous diluent to the vapor phase.

21. The method of claim 19 wherein the composition of the vapor phase above the resultant solution is maintained at a noninflammable composition by refrigeration of the resultant solution with a liquefied-gas refrigerant.

22. The method of claim 19 wherein the composition of the vapor phase above the solution is maintained at a noninflammable composition by providing a follower for the surface of the resultant solution selected from the class consisting of minute plastic bubbles and thin plastic sheets.

23. A package comprising a receptacle, a partition effectively dividing the receptacle into two compartments, one of the compartments of the receptacle containing liquid oxygen and the other compartment of the receptacle containing at least one fuel material selected from the class consisting of methane, ethane and propane, and means for removing at least a portion of the partition thereby allowing the contents of the two compartments to mix and form a solution of the fuel material in the liquid oxygen.

24. A package comprising a receptacle, a partition effectively dividing the receptacle into two compartments, one of the compartments of the receptacle containing liquid oxygen and the other compartment of the receptacle containing methane, and means for removing at least a portion of the partition thereby allowing the con-

tents of the two compartments to mix and form a solution of methane in liquid oxygen.

25. A method of storing and handling an explosive which consists essentially of at least one fuel material selected from the class consisting of methane, ethane and propane dissolved in liquid oxygen comprising reducing the explosion hazard by maintaining the concentration of fuel material in the liquid oxygen in a range effective to produce an explosive and prevent the formation of a second nongaseous phase comprising fuel material, the resulting solution of fuel material dissolved in liquid oxygen being at a temperature below its critical temperature and above  $-363^{\circ}$  F. and containing based upon the total molar amount of fuel material and liquid oxygen up to about 75 mol percent of methane, up to about 40 mol percent of ethane and up to about 7 mol percent of propane.

26. The method of claim 25 wherein the vapor phase above the solution is noninflammable, the concentration of fuel material in the vapor phase being less than 5.4 mol percent.

27. A method of storing and handling an explosive which consists essentially of methane dissolved in liquid oxygen comprising reducing the explosion hazard by maintaining the concentration of methane in the liquid oxygen in a range effective to produce an explosive and prevent the formation of a second nongaseous phase comprising methane, the resulting solution of methane dissolved in liquid oxygen being at a temperature below its critical temperature and above  $-363^{\circ}$  F. and containing 5-75 mol percent methane based upon the total molar amount of methane and liquid oxygen.

28. The method of claim 27 wherein the concentration of methane is about 33 mol percent.

29. The method of claim 27 wherein the vapor phase above the solution is noninflammable, the concentration of methane in the vapor phase being less than 5.4 mol percent.

40

#### References Cited in the file of this patent

#### UNITED STATES PATENTS

|           |         |               |
|-----------|---------|---------------|
| 1,508,185 | Haynes  | Sept. 9, 1924 |
| 2,532,708 | Goddard | Dec. 5, 1950  |
| 2,584,875 | Hasche  | Feb. 5, 1952  |

#### OTHER REFERENCES

"Astronautics," Aug.-Sept. 1932, No. 22, page 4.